



US006835779B2

(12) **United States Patent**  
**Voorheis et al.**

(10) **Patent No.:** **US 6,835,779 B2**  
(b5) **Date of Patent:** **Dec. 28, 2004**

(54) **GOLF BALLS CONTAINING A HALOGENATED ORGANOSULFUR COMPOUND AND RESILIENT REGRIND**

(75) Inventors: **Peter Voorheis**, Fall River, MA (US); **Ryan W Bosanko**, Mattapoisett, MA (US); **David A Bulpett**, Boston, MA (US); **Derek A Ladd**, Fairhaven, MA (US); **Murali Rajagopalan**, South Dartmouth, MA (US)

(73) Assignee: **Acushnet Company**, Fairhaven, MA (US)

(\*) Notice: Subject to any disclaimer, the term of this patent is extended or adjusted under 35 U.S.C. 154(b) by 59 days.

(21) Appl. No.: **10/308,537**

(22) Filed: **Dec. 3, 2002**

(65) **Prior Publication Data**

US 2003/0130063 A1 Jul. 10, 2003

**Related U.S. Application Data**

(63) Continuation-in-part of application No. 09/951,963, filed on Sep. 13, 2001, now Pat. No. 6,635,716.  
(51) **Int. Cl.** <sup>7</sup> **A63B 37/06**  
(52) **U.S. Cl.** **525/193; 525/261; 525/274; 473/377**  
(58) **Field of Search** **525/193, 261, 525/274; 473/377, 372**

(56) **References Cited**

**U.S. PATENT DOCUMENTS**

|             |         |                        |           |
|-------------|---------|------------------------|-----------|
| 5,252,652 A | 10/1993 | Egashira et al. ....   | 524/392   |
| 5,574,107 A | 11/1996 | Hiraoka et al. ....    | 525/193   |
| 5,589,546 A | 12/1996 | Hiraoka et al. ....    | 525/193   |
| 5,605,968 A | 2/1997  | Egashira et al. ....   | 525/221   |
| 5,697,856 A | 12/1997 | Moriyama et al. ....   | 473/374   |
| 5,711,723 A | 1/1998  | Hiraoka et al. ....    | 473/374   |
| 5,776,012 A | 7/1998  | Moriyama et al. ....   | 473/372   |
| 5,779,563 A | 7/1998  | Yamagishi et al. ....  | 473/371   |
| 5,816,944 A | 10/1998 | Asakura et al. ....    | 473/372   |
| 5,826,944 A | 10/1998 | Beneker et al. ....    | 297/440.2 |
| 5,872,185 A | 2/1999  | Ichikawa et al. ....   | 525/93    |
| 5,877,264 A | 3/1999  | Logothetis et al. .... | 526/86    |
| 5,919,101 A | 7/1999  | Yokota et al. ....     | 473/374   |
| 5,929,171 A | 7/1999  | Sano et al. ....       | 525/261   |
| 5,977,264 A | 11/1999 | Ichikawa et al. ....   | 525/329.9 |
| 5,994,472 A | 11/1999 | Egashira et al. ....   | 525/221   |
| 6,120,392 A | 9/2000  | Kashiwagi et al. ....  | 473/374   |
| 6,121,357 A | 9/2000  | Yokota ....            | 524/406   |
| 6,126,558 A | 10/2000 | Higuchi et al. ....    | 473/374   |
| 6,129,640 A | 10/2000 | Higuchi et al. ....    | 473/374   |
| 6,135,898 A | 10/2000 | Higuchi et al. ....    | 473/374   |

|                   |         |                      |         |
|-------------------|---------|----------------------|---------|
| 6,139,447 A       | 10/2000 | Ohama .....          | 473/378 |
| 6,162,135 A       | 12/2000 | Bulpett et al. ....  | 473/373 |
| 6,174,247 B1      | 1/2001  | Higuchi et al. ....  | 473/374 |
| 6,184,301 B1      | 2/2001  | Shindo et al. ....   | 525/261 |
| 6,210,292 B1      | 4/2001  | Higuchi et al. ....  | 473/374 |
| 6,213,896 B1      | 4/2001  | Higuchi et al. ....  | 473/374 |
| 6,231,460 B1      | 5/2001  | Higuchi et al. ....  | 473/374 |
| 6,241,625 B1      | 6/2001  | Yokota et al. ....   | 473/373 |
| 6,244,978 B1      | 6/2001  | Higuchi et al. ....  | 473/374 |
| 6,248,028 B1      | 6/2001  | Higuchi et al. ....  | 473/374 |
| 6,267,692 B1      | 7/2001  | Higuchi et al. ....  | 473/365 |
| 6,287,218 B1      | 9/2001  | Ohama .....          | 473/377 |
| 6,291,592 B1      | 9/2001  | Bulpett et al. ....  | 525/248 |
| 6,299,551 B1      | 10/2001 | Higuchi et al. ....  | 473/374 |
| 6,494,793 B1 *    | 12/2002 | Ohama .....          | 473/371 |
| 6,561,926 B2 *    | 5/2003  | Hayashi et al. ....  | 473/372 |
| 2001/0011045 A1   | 8/2001  | Takemura et al. .... | 473/371 |
| 2001/0016522 A1   | 8/2001  | Watanabe et al. .... | 473/371 |
| 2001/0018374 A1   | 8/2001  | Ichikawa et al. .... | 473/367 |
| 2001/0031669 A1   | 10/2001 | Ohama .....          | 473/371 |
| 2001/0031673 A1   | 10/2001 | Watanabe .....       | 473/378 |
| 2002/0065149 A1 * | 5/2002  | Tzivanis et al. .... | 473/371 |

\* cited by examiner

*Primary Examiner*—David J. Buttner

(74) *Attorney, Agent, or Firm*—William B. Lacy

(57) **ABSTRACT**

A golf ball consisting of a core and a cover. The core has a diameter of between about 1.54 and about 1.58 inches and a compression of between about 22 and about 50. Additionally, the core includes a polybutadiene rubber having a Mooney viscosity of less than about 50 and a halogenated organosulfur compound present in an amount of at least about 2.2 parts per hundred parts of polybutadiene rubber, the halogenated organosulfur compound having the formula:



where R<sub>1</sub>–R<sub>5</sub> are C<sub>1</sub>–C<sub>8</sub> alkyl groups; halogen groups; thiol groups; carboxylated groups; sulfonated groups; or hydrogen; and a regrind filler present in an amount of from about 5 parts to about 26.5 parts per hundred parts of polybutadiene rubber. The cover has a thickness of between about 0.05 inches and about 0.1 inches and consisting essentially of a first ionomer material and a second ionomer material. The golf ball has a coefficient of restitution of at least about 0.813 when measured at 125 ft/s.

**19 Claims, No Drawings**

1

**GOLF BALLS CONTAINING A HALOGENATED ORGANOSULFUR COMPOUND AND RESILIENT REGRIND**

**CROSS-REFERENCE To RELATED APPLICATIONS**

This application is a continuation-in-part of U.S. patent application Ser. No. 09/951,963, filed Sep. 13, 2001, now U.S. Pat. No. 6,635,716, the disclosure of which is incorporated herein, in its entirety, by express reference thereto.

**FIELD OF THE INVENTION**

This invention relates generally to golf balls and, in particular, golf ball cores formed of a polymer composition including a halogenated organosulfur compound and resilient regrind.

**BACKGROUND**

Conventional golf balls can be divided into two general classes: solid and wound. Solid golf balls include one-piece, two-piece (i.e., solid core and a cover), and multi-layer (i.e., solid core of one or more layers and/or a cover of one or more layers) golf balls. Wound golf balls typically include a solid, hollow, or fluid-filled center, surrounded by a tensioned elastomeric material, and a cover. Solid balls have traditionally been considered longer and more durable than wound balls, but also lack a particular "feel" provided by the wound construction.

By altering ball construction and composition, manufacturers can vary a wide range of playing characteristics, such as compression, velocity, and spin, each of which can be optimized for various playing abilities. One golf ball component, in particular, that many manufacturers are continually looking to improve is the center or core. The core becomes the "engine" of the golf ball when hit with a club head. Generally, golf ball cores and/or centers are constructed with a polybutadiene-based polymer composition. Compositions of this type are constantly being altered in an effort to provide a higher coefficient of restitution ("COR") while at the same time resulting in a lower compression which, in turn, can lower the golf ball spin rate, provide better "feel," or both. This is a difficult task, however, given the physical limitations of currently-available polymers. As such, there remains a need for novel and improved golf ball core compositions.

It has been determined that, upon that addition of a halogenated organosulfur compound or the salts thereof, in particular, pentachlorothiophenol ("PCTP") salt, to polybutadiene rubber compositions, that golf ball cores may be constructed that exhibit increased COR, decreased compression, or both. The present invention is, therefore, directed to golf ball centers and cores that include a halogenated organosulfur compound, or a salt thereof, for embodiments such as these.

**SUMMARY OF THE INVENTION**

The present invention is directed to a two-piece golf ball including a core having a diameter of between about 1.54 and about 1.58 inches and a compression of between about 22 and about 50, the core including a polybutadiene rubber having a Mooney viscosity of less than about 50 and a halogenated organosulfur compound present in an amount of at least about 2.2 parts per hundred parts of polybutadiene rubber, the halogenated organosulfur compound having the formula:

2



5

10

where  $R_1-R_5$  are  $C_1-C_8$  alkyl groups; halogen groups; thiol groups; carboxylated groups; sulfonated groups; or hydrogen; and a regrind filler present in an amount of from about 5 parts to about 26.5 parts per hundred parts of polybutadiene rubber; and a cover having a thickness of between about 0.05 inches and about 0.1 inches, the cover including a first ionomer material and a second ionomer material; wherein the golf ball has a coefficient of restitution of at least about 0.813 when measured at 125 ft/s.

15

The regrind is vulcanized polybutadiene rubber that contains a substantially greater amount of the trans-polybutadiene isomer than prior to vulcanization and is preferably present in an amount of from about 10.6 parts to about 19.7 parts per hundred parts of polybutadiene rubber. The core of the golf ball preferably has a diameter of between about 1.54 and about 1.57 inches. The amount of the trans-polybutadiene isomer in the vulcanized polybutadiene rubber is between about 10% and about 60%.

20

The polybutadiene composition further comprises an  $\alpha,\beta$ -unsaturated carboxylic acid or a metal salt thereof, an organic peroxide, and a second filler. Preferably, the  $\alpha,\beta$ -unsaturated carboxylic acid or a metal salt thereof is present in an amount greater than about 30 parts per hundred parts of polybutadiene rubber. More preferably, the  $\alpha,\beta$ -unsaturated carboxylic acid or a metal salt thereof is present in an amount greater than about 41 parts per hundred parts of polybutadiene rubber. The at least one of the first and second ionomer materials may include  $\alpha,\beta$ -unsaturated carboxylic acid groups, or the salts thereof, that have been partially- or fully-neutralized by organic fatty acids.

25

In a preferred embodiment, the halogenated organosulfur compound is present in an amount between about 2.2 parts and about 5 parts. Ideally, the halogenated organosulfur compound is selected from the group consisting of pentachlorothiophenol or a metal salt of pentachlorothiophenol. If the metal salt is selected, preferably the metal salt is selected from the group consisting of zinc, calcium, magnesium, sodium, and lithium and, most preferably, the metal salt is zinc.

30

The first and second ionomer materials include copolymers or terpolymers of ethylene and methacrylic acid or acrylic acid partially- or fully-neutralized with salts of zinc, sodium, lithium, magnesium, potassium, calcium, manganese, or nickel. Additionally, the core includes between about 1 part and 50 parts vulcanized polybutadiene rubber per hundred parts first polybutadiene rubber and the cover has a  $\tan^*$  of between about 0.07 and about 0.09 measured over the range of  $-30^\circ C$ . to  $20^\circ C$ .

35

Preferably, the first ionomer material present in an amount between about 45% and about 55% and the second ionomer material present in an amount between about 55% and about 45%. Additionally, the core preferably has a surface hardness and a geometric center hardness that differs from the surface hardness by between about 15 Shore D and about 20 Shore D. In a preferred embodiment, the golf ball has a coefficient of restitution of between about 0.813 and about 0.823.

The present invention is also directed to a golf ball consisting of a core having a diameter of between about 1.54 and about 1.57 inches and a compression of between about 22 and about 50, the core comprising a first polybutadiene rubber having a Mooney viscosity of less than about 50 and a halogenated organosulfur compound or the salt thereof, the halogenated organosulfur compound having the formula:



where  $R_1-R_5$  are  $C_1-C_8$  alkyl groups; halogen groups; thiol groups; carboxylated groups; sulfonated groups; or hydrogen; and regrind filler present in an amount of from about 10.6 parts to about 19.7 parts per hundred parts of polybutadiene rubber; and a cover having a thickness of between about 0.05 inches and about 0.1 inches, the cover consisting essentially of a first ionomeric material and a second ionomeric material; wherein the golf ball has a coefficient of restitution of at least about 0.813 when measured at 125 ft/s.

The present invention is further directed to a golf ball including a core having a diameter of between about 1.54 and about 1.61 inches and a compression of between about 22 and about 70, the core including 1,4-polybutadiene having a cis-structure of at least about 95% and a Mooney viscosity of less than about 50; and a filler comprising a trans-regrind polybutadiene rubber having a trans-isomer content of between about 10% and about 60% and present in an amount of from about 5 parts to about 26.5 parts per hundred parts of cis-1,4-polybutadiene rubber; and a cover having a thickness of between about 0.05 inches and about 0.1 inches, the cover consisting essentially of a first ionomeric material and a second ionomeric material; wherein the golf ball has a coefficient of restitution of between about 0.801 and 0.823 when measured at an incoming velocity of 125 ft/s.

#### DETAILED DESCRIPTION OF THE PREFERRED EMBODIMENTS

The golf ball cores of the present invention may comprise any of a variety of constructions but preferably includes a core and a cover surrounding the core. The core and/or the cover may have more than one layer and an intermediate layer may be disposed between the core and the cover of the golf ball. For example, the core of the golf ball may comprise a conventional center surrounded by an intermediate or outer core layer disposed between the center and the inner cover layer. The core may be a single layer or may comprise a plurality of layers. The innermost portion of the core may be solid or it may be a liquid filled sphere, but preferably it is solid. As with the core, the intermediate layer or outer core layer may also comprise a plurality of layers. The core may also comprise a solid or liquid filled center around which many yards of a tensioned elastomeric material are wound.

The materials for solid cores include compositions having a base rubber, a crosslinking agent, a filler, a halogenated organosulfur compound, and a co-crosslinking or initiator agent. The base rubber typically includes natural or synthetic rubbers. A preferred base rubber is 1,4-polybutadiene having a cis-structure of at least 40%, more preferably at least about

90%, and most preferably at least about 95%. Two non-limiting, but preferred examples, of a preferred base rubber include CARIFLEX® 1220, commercially-available from Shell, and KINEX® 7245, commercially-available from Goodyear. Most preferably, the base rubber comprises high-Mooney-viscosity rubber. Preferably, the base rubber has a Mooney viscosity greater than about 35, more preferably greater than about 50. Preferably, the polybutadiene rubber has a molecular weight greater than about 400,000 and a polydispersity of no greater than about 2, more preferably between about 2 and about 1. Examples of desirable polybutadiene rubbers include BUNA® CB22 and BUNA® CB23, commercially available from Bayer of Akron, Ohio; UBEPOL® 360L and UBEPOL® 150L, commercially available from UBE Industries of Tokyo, Japan; and CARI-FLEX® BCP820 and CARI-FLEX® BCP824, commercially available from Shell of Houston, Tex. If desired, the polybutadiene can also be mixed with other elastomers known in the art such as natural rubber, polyisoprene rubber and/or styrene-butadiene rubber in order to modify the properties of the core.

The crosslinking agent includes a metal salt, such as a zinc salt or a magnesium unsaturated fatty acid, such as acrylic or methacrylic acid, having 3 to 8 carbon atoms. Examples include, but are not limited to, one or more metal salt diacrylates, dimethacrylates, and monomethacrylates, wherein the metal is magnesium, calcium, zinc, aluminum, sodium, lithium, or nickel. Preferred acrylates include zinc acrylate, zinc diacrylate, zinc methacrylate, zinc dimethacrylate, and mixtures thereof. The crosslinking agent is typically present in an amount greater than about 10 parts per hundred ("pph") parts of the base polymer, preferably from about 20 to 40 pph of the base polymer, more preferably from about 25 to 35 pph of the base polymer.

The initiator agent can be any known polymerization initiator which decomposes during the cure cycle. Suitable initiators include organic peroxide compounds, such as dicumyl peroxide;  $\alpha,\alpha$ -bis(t-butylperoxy) 3,3,5-trimethyl cyclohexane;  $\alpha,\alpha$ -bis(t-butylperoxy)diisopropylbenzene; 2,5-dimethyl-2,5 di-(t-butylperoxy)hexane; di-t-butyl peroxide; and mixtures thereof. Other examples include, but are not limited to, VAROX® 231XL and VAROX® DCP-R, commercially available from Elf Atochem of Philadelphia, Pa.; PERKODOX® BC and PERKODOX® 14, commercially available from Akzo Nobel of Chicago, Ill.; and ELASTOCHEM® DCP-70, commercially available from Rhein Chemie of Trenton, N.J.

It is well known that peroxides are available in a variety of forms having different activity. The activity is typically defined by the "active oxygen content." For example, PERKODOX® BC peroxide is 98% active and has an active oxygen content of 5.80%, whereas PERKODOX® DCP-70 is 70% active and has an active oxygen content of 4.18%. If the peroxide is present in pure form, it is preferably present in an amount of at least about 0.25 pph, more preferably between about 0.35 pph and about 2.5 pph, and most preferably between about 0.5 pph and about 2 pph. Peroxides are also available in concentrate form, which are well-known to have differing activities, as described above. In this case, if concentrate peroxides are employed in the present invention, one skilled in the art would know that the concentrations suitable for pure peroxides are easily adjusted for concentrate peroxides by dividing by the activity. For example, 2 pph of a pure peroxide is equivalent 4 pph of a concentrate peroxide that is 50% active (i.e., 2 divided by 0.5=4).

The halogenated organosulfur compounds of the present invention include, but are not limited to those having the following general formula:



where R<sub>1</sub>–R<sub>5</sub> can be C<sub>1</sub>–C<sub>8</sub> alkyl groups; halogen groups; thiol groups (—SH), carboxylated groups; sulfonated groups; and hydrogen; in any order; and also pentachlorothiophenol; 2-fluorothiophenol; 3-fluorothiophenol; 4-fluorothiophenol; 2,3-fluorothiophenol; 2,4-fluorothiophenol; 3,4-fluorothiophenol; 3,5-fluorothiophenol; 2,3,4-fluorothiophenol; 3,4,5-fluorothiophenol; 2,3,4,5-tetrafluorothiophenol; 2,3,5,6-tetrafluorothiophenol; 4-chlorotetrafluorothiophenol; pentachlorothiophenol; 2-chlorothiophenol; 3-chlorothiophenol; 4-chlorothiophenol; 2,3-chlorothiophenol; 2,4-chlorothiophenol; 3,4-chlorothiophenol; 3,5-chlorothiophenol; 2,3,4-chlorothiophenol; 3,4,5-chlorothiophenol; 2,3,4,5-tetrachlorothiophenol; 2,3,5,6-tetrachlorothiophenol; pentabromothiophenol; 2-bromothiophenol; 3-bromothiophenol; 4-bromothiophenol; 2,3-bromothiophenol; 2,4-bromothiophenol; 3,4-bromothiophenol; 3,5-bromothiophenol; 2,3,4-bromothiophenol; 3,4,5-bromothiophenol; 2,3,4,5-tetrabromothiophenol; 2,3,5,6-tetrabromothiophenol; pentaiodothiophenol; 2-iodothiophenol; 3-iodothiophenol; 4-iodothiophenol; 2,3-iodothiophenol; 2,4-iodothiophenol; 3,4-iodothiophenol; 3,5-iodothiophenol; 2,3,4-iodothiophenol; 3,4,5-iodothiophenol; 2,3,5,6-tetraiodothiophenol; 2,3,5,6-tetraiodothiophenol; and their zinc salts. Preferably, the halogenated organosulfur compound is pentachlorothiophenol, which is commercially available in neat form or under the tradename STRUKTOL®, a clay-based carrier containing the sulfur compound pentachlorothiophenol loaded at 45 percent (correlating to 2.4 parts PCTP). STRUKTOL® is commercially available from Struktol Company of America of Stow, Ohio. PCTP is commercially available in neat form from eChinachem of San Francisco, Calif. and in the salt form from eChinachem of San Francisco, Calif. Most preferably, the halogenated organosulfur compound is the zinc salt of pentachlorothiophenol, which is commercially available from eChinachem of San Francisco, Calif. The halogenated organosulfur compounds of the present invention are preferably present in an amount greater than about 2.2 pph, more preferably between about 2.3 pph and about 5 pph, and most preferably between about 2.3 and about 4 pph.

Fillers typically include materials such as tungsten, zinc oxide, barium sulfate, silica, calcium carbonate, zinc carbonate, metals, metal oxides and salts, regrind (recycled core material typically ground to about 30 mesh particle), high-Mooney-viscosity rubber regrind, trans-regrind core material (recycled core material containing high trans-isomer of polybutadiene, prepared as described below), and the like. When trans-regrind is present, the amount of trans-isomer is preferably between about 10% and about 60%. In a preferred embodiment of the invention, the core comprises polybutadiene having a cis-isomer content of greater than about 95% and trans-regrind core material

(already vulcanized) as a filler. Any particle size trans-regrind core material is sufficient, but is preferably less than about 125  $\mu\text{m}$ .

Fillers added to one or more portions of the golf ball typically include processing aids or compounds to affect rheological and mixing properties, density-modifying fillers, tear strength, or reinforcement fillers, and the like. The fillers are generally inorganic, and suitable fillers include numerous metals or metal oxides, such as zinc oxide and tin oxide, as well as barium sulfate, zinc sulfate, calcium carbonate, barium carbonate, clay, tungsten carbide, an array of silicas, and mixtures thereof. Fillers may also include various foaming agents or blowing agents which may be readily selected by one of ordinary skill in the art. Fillers may include polymeric, ceramic, metal, and glass microspheres may be solid or hollow, and filled or unfilled. Fillers are typically also added to one or more portions of the golf ball to modify the density thereof to conform to uniform golf ball standards. Fillers may also be used to modify the weight of the center or at least one additional layer for specialty balls, e.g., a lower weight ball is preferred for a player having a low swing speed.

The invention also includes a method to convert the cis-isomer of the polybutadiene resilient polymer component to the trans-isomer during a molding cycle and to form a golf ball. A variety of methods and materials suitable for cis-to-trans conversion have been disclosed in U.S. Pat. No. 6,162,135 and U.S. application Ser. No. 09/461,736, filed Dec. 16, 1999; Ser. No. 09/458,676, filed Dec. 10, 1999; and Ser. No. 09/461,421, filed Dec. 16, 1999, each of which are incorporated herein, in their entirety, by reference.

The materials used in forming either the golf ball center or any portion of the core, in accordance with the invention, may be combined to form a mixture by any type of mixing known to one of ordinary skill in the art. Suitable types of mixing include single pass and multi-pass mixing. Suitable mixing equipment is well known to those of ordinary skill in the art, and such equipment may include a Banbury mixer, a two-roll mill, or a twin screw extruder.

Conventional mixing speeds for combining polymers are typically used. The mixing temperature depends upon the type of polymer components, and more importantly, on the type of free-radical initiator. Suitable mixing speeds and temperatures are well-known to those of ordinary skill in the art, or may be readily determined without undue experimentation.

The mixture can be subjected to, e.g., a compression or injection molding process, to obtain solid spheres for the center or hemispherical shells for forming an intermediate layer. The temperature and duration of the molding cycle are selected based upon reactivity of the mixture. The molding cycle may have a single step of molding the mixture at a single temperature for a fixed time duration. The molding cycle may also include a two-step process, in which the polymer mixture is held in the mold at an initial temperature for an initial duration of time, followed by holding at a second, typically higher temperature for a second duration of time. In a preferred embodiment of the current invention, a single-step cure cycle is employed. The materials used in forming either the golf ball center or any portion of the core, in accordance with the invention, may be combined to form a golf ball by an injection molding process, which is also well-known to one of ordinary skill in the art. Although the curing time depends on the various materials selected, those of ordinary skill in the art will be readily able to adjust the curing time upward or downward based on the particular materials used and the discussion herein.

Properties that are desirable for the cover include good moldability, high abrasion resistance, high tear strength, high resilience, and good mold release. The cover typically has a thickness to provide sufficient strength, good performance characteristics, and durability. The cover preferably has a thickness of less than about 0.1 inches, more preferably, less than about 0.05 inches, and most preferably, between about 0.02 inches and about 0.04 inches. The invention is particularly directed towards a multilayer golf ball which comprises a core, an inner cover layer, and an outer cover layer. In this embodiment, preferably, at least one of the inner and outer cover layer has a thickness of less than about 0.05 inches, more preferably between about 0.02 inches and about 0.04 inches. Most preferably, the thickness of either layer is about 0.03 inches.

When the golf ball of the present invention includes an inner cover layer, this layer can include any materials known to those of ordinary skill in the art, including thermoplastic and thermosetting material, but preferably the inner cover can include any suitable materials, such as ionic copolymers of ethylene and an unsaturated monocarboxylic acid which are available under the trademark SURLYN® of E.I. DuPont de Nemours & Co., of Wilmington, Del., or IOTEK® or ESCOR® of Exxon. These are copolymers or terpolymers of ethylene and methacrylic acid or acrylic acid partially neutralized with salts of zinc, sodium, lithium, magnesium, potassium, calcium, manganese, nickel or the like, in which the salts are the reaction product of an olefin having from 2 to 8 carbon atoms and an unsaturated monocarboxylic acid having 3 to 8 carbon atoms. The carboxylic acid groups of the copolymer may be totally or partially neutralized and might include methacrylic, crotonic, maleic, fumaric or itaconic acid.

This golf ball can likewise include one or more homopolymeric or copolymeric inner cover materials, such as:

- (1) Vinyl resins, such as those formed by the polymerization of vinyl chloride, or by the copolymerization of vinyl chloride with vinyl acetate, acrylic esters or vinylidene chloride;
- (2) Polyolefins, such as polyethylene, polypropylene, polybutylene and copolymers such as ethylene methylacrylate, ethylene ethylacrylate, ethylene vinyl acetate, ethylene methacrylic or ethylene acrylic acid or propylene acrylic acid and copolymers and homopolymers produced using a single-site catalyst or a metallocene catalyst;
- (3) Polyurethanes, such as those prepared from polyols and diisocyanates or polyisocyanates and those disclosed in U.S. Pat. No. 5,334,673;
- (4) Polyureas, such as those disclosed in U.S. Pat. No. 5,484,870;
- (5) Polyamides, such as poly(hexamethylene adipamide) and others prepared from diamines and dibasic acids, as well as those from amino acids such as poly (caprolactam), and blends of polyamides with SURLYN®, polyethylene, ethylene copolymers, ethyl-propylene-non-conjugated diene terpolymer, and the like;
- (6) Acrylic resins and blends of these resins with poly vinyl chloride, elastomers, and the like;
- (7) Thermoplastics, such as urethanes; olefinic thermoplastic rubbers, such as blends of polyolefins with ethylene-propylene-non-conjugated diene terpolymer; block copolymers of styrene and butadiene, isoprene or ethylene-butylene rubber; or copoly(ether-amide), such as PEBAK®, sold by ELF Atochem of Philadelphia, Pa.;

(8) Polyphenylene oxide resins or blends of polyphenylene oxide with high impact polystyrene as sold under the trademark NORYL® by General Electric Company of Pittsfield, Mass.;

(9) Thermoplastic polyesters, such as polyethylene terephthalate, polybutylene terephthalate, polyethylene terephthalate/glycol modified and elastomers sold under the trademarks HYTREL® by E.I. DuPont de Nemours & Co. of Wilmington, Del., and LOMOD® by General Electric Company of Pittsfield, Mass.;

(10) Blends and alloys, including polycarbonate with acrylonitrile butadiene styrene, polybutylene terephthalate, polyethylene terephthalate, styrene maleic anhydride, polyethylene, elastomers, and the like, and polyvinyl chloride with acrylonitrile butadiene styrene or ethylene vinyl acetate or other elastomers; and

(11) Blends of thermoplastic rubbers with polyethylene, propylene, polyacetal, nylon, polyesters, cellulose esters, and the like.

Preferably, the inner cover includes polymers, such as ethylene, propylene, butene-1 or hexane-1 based homopolymers or copolymers including functional monomers, such as acrylic and methacrylic acid and fully or partially neutralized ionomer resins and their blends, methyl acrylate, methyl methacrylate homopolymers and copolymers, imidized, amino group containing polymers, polycarbonate, reinforced polyamides, polyphenylene oxide, high impact polystyrene, polyether ketone, polysulfone, poly(phenylene sulfide), acrylonitrile-butadiene, acrylic-styrene-acrylonitrile, poly(ethylene terephthalate), poly(butylene terephthalate), poly(ethylene vinyl alcohol), poly(tetrafluoroethylene) and their copolymers including functional comonomers, and blends thereof. Suitable cover compositions also include a polyether or polyester thermoplastic urethane, a thermoset polyurethane, a low modulus ionomer, such as acid-containing ethylene copolymer ionomers, including E/X/Y terpolymers where E is ethylene, X is an acrylate or methacrylate-based softening comonomer

present in about 0 to 50 weight percent and Y is acrylic or methacrylic acid present in about 5 to 35 weight percent. Preferably, the acrylic or methacrylic acid is present in about 8 to 35 weight percent, more preferably 8 to 25 weight percent, and most preferably 8 to 20 weight percent.

Any of the inner or outer cover layers may also be formed from polymers containing  $\alpha,\beta$ -unsaturated carboxylic acid groups, or the salts thereof, that have been 100 percent neutralized by organic fatty acids. The acid moieties of the highly-neutralized polymers ("HNP"), typically ethylene-based ionomers, are preferably neutralized greater than about 70%, more preferably greater than about 90%, and most preferably at least about 100%. The HNP's can be also be blended with a second polymer component, which, if containing an acid group, may be neutralized in a conventional manner, by the organic fatty acids of the present invention, or both. The second polymer component, which may be partially or fully neutralized, preferably comprises ionomeric copolymers and terpolymers, ionomer precursors, thermoplastics, polyamides, polycarbonates, polyesters, polyurethanes, polyureas, thermoplastic elastomers, polybutadiene rubber, balata, metallocene-catalyzed polymers (grafted and non-grafted), single-site polymers, high-crystalline acid polymers, cationic ionomers, and the like.

The acid copolymers can be described as E/X/Y copolymers where E is ethylene, X is an  $\alpha,\beta$ -ethylenically unsaturated carboxylic acid, and Y is a softening comonomer. In a preferred embodiment, X is acrylic or methacrylic acid and

Y is a C<sub>1-8</sub> alkyl acrylate or methacrylate ester. X is preferably present in an amount from about 1 to about 35 weight percent of the polymer, more preferably from about 5 to about 30 weight percent of the polymer, and most preferably from about 10 to about 20 weight percent of the polymer. Y is preferably present in an amount from about 0 to about 50 weight percent of the polymer, more preferably from about 5 to about 25 weight percent of the polymer, and most preferably from about 10 to about 20 weight percent of the polymer.

The organic acids are aliphatic, mono-functional (saturated, unsaturated, or multi-unsaturated) organic acids. Salts of these organic acids may also be employed. The salts of organic acids of the present invention include the salts of barium, lithium, sodium, zinc, bismuth, chromium, cobalt, copper, potassium, strontium, titanium, tungsten, magnesium, cesium, iron, nickel, silver, aluminum, tin, or calcium, salts of fatty acids, particularly stearic, behenic, erucic, oleic, linoelic or dimerized derivatives thereof. It is preferred that the organic acids and salts of the present invention be relatively non-migratory (they do not bloom to the surface of the polymer under ambient temperatures) and non-volatile (they do not volatilize at temperatures required for melt-blending).

Thermoplastic polymer components, such as copolyetheresters, copolyesteresters, copolyetheramides, elastomeric polyolefins, styrene diene block copolymers and their hydrogenated derivatives, copolyesteramides, thermoplastic polyurethanes, such as copolyetherurethanes, copolyesterurethanes, copolyureaurethanes, epoxy-based polyurethanes, polycaprolactone-based polyurethanes, polyureas, and polycarbonate-based polyurethanes fillers, and other ingredients, if included, can be blended in either before, during, or after the acid moieties are neutralized, thermoplastic polyurethanes.

Examples of these materials are disclosed in U.S. patent application Publication Nos. 2001/0018375 and 2001/0019971, which are incorporated herein in their entirety by express reference thereto.

While the outer cover may be formed of any of the above-listed materials, the outer cover preferably includes a polyurethane, polyurea, or epoxy composition, generally comprising the reaction product of at least one polyisocyanate, polyol, and at least one curing agent. Any polyisocyanate available to one of ordinary skill in the art is suitable for use according to the invention. Exemplary polyisocyanates include, but are not limited to, 4,4'-diphenylmethane diisocyanate ("MDI"); polymeric MDI; carbodiimide-modified liquid MDI; 4,4'-dicyclohexylmethane diisocyanate ("H<sub>12</sub>-MDI"); p-phenylene diisocyanate ("PPDI"); m-phenylene diisocyanate ("MPDI"); toluene diisocyanate ("TDI"); 3,3'-dimethyl-4,4'-biphenylene diisocyanate ("TODI"); isophorone diisocyanate ("IPDI"); hexamethylene diisocyanate ("HDI"); naphthalene diisocyanate ("NDI"); xylene diisocyanate ("XDI"); p-tetramethylxylene diisocyanate ("p-TMXDI"); m-tetramethylxylene diisocyanate ("m-TMXDI"); ethylene diisocyanate; propylene-1,2-diisocyanate; tetramethylene-1,4-diisocyanate; cyclohexyl diisocyanate; 1,6-hexamethylene-diisocyanate ("HDI"); dodecane-1,12-diisocyanate; cyclobutane-1,3-diisocyanate; cyclohexane-1,3-diisocyanate; cyclohexane-1,4-diisocyanate; 1-isocyanato-3,3,5-trimethyl-5-isocyanatomethylcyclohexane; methyl cyclohexylene diisocyanate; triisocyanate of HDI; triisocyanate of 2,4,4-trimethyl-1,6-hexane diisocyanate ("TMDI"); tetracene diisocyanate; naphthalene diisocyanate; anthracene diisocyanate;

anate; isocyanurate of toluene diisocyanate; uretdione of hexamethylene diisocyanate; and mixtures thereof. Preferably, the polyisocyanate includes MDI, PPDI, TDI, or a mixture thereof, and more preferably, the polyisocyanate includes MDI. It should be understood that, as used herein, the term "MDI" includes 4,4'-diphenylmethane diisocyanate, polymeric MDI, carbodiimide-modified liquid MDI, and mixtures thereof and, additionally, that the diisocyanate employed may be "low free monomer," understood by one of ordinary skill in the art to have lower levels of "free" monomer isocyanate groups, typically less than about 0.1% free monomer groups. Examples of "low free monomer" diisocyanates include, but are not limited to Low Free Monomer MDI, Low Free Monomer TDI, and Low Free Monomer PPDI.

The at least one polyisocyanate should have less than about 14% unreacted NCO groups. Preferably, the at least one polyisocyanate has no greater than about 7.5% NCO, and more preferably, less than about 7.0%.

Any polyol available to one of ordinary skill in the art is suitable for use according to the invention. Exemplary polyols include, but are not limited to, polyether polyols, hydroxy-terminated polybutadiene (including partially/fully hydrogenated derivatives), polyester polyols, polycaprolactone polyols, and polycarbonate polyols. In one preferred embodiment, the polyol includes polyether polyol. Examples include, but are not limited to, polytetramethylene ether glycol ("PTMEG"), polyethylene propylene glycol, polyoxypropylene glycol, and mixtures thereof. The hydrocarbon chain can have saturated or unsaturated bonds and substituted or unsubstituted aromatic and cyclic groups. Preferably, the polyol of the present invention includes PTMEG.

Suitable polyester polyols include, but are not limited to, polyethylene adipate glycol; polybutylene adipate glycol; polyethylene propylene adipate glycol; o-phthalate-1,6-hexanediol; poly(hexamethylene adipate)glycol; and mixtures thereof. The hydrocarbon chain can have saturated or unsaturated bonds, or substituted or unsubstituted aromatic and cyclic groups.

Suitable polycaprolactone polyols include, but are not limited to, 1,6-hexanediol-initiated polycaprolactone, diethylene glycol initiated polycaprolactone, trimethylol propane initiated polycaprolactone, neopentyl glycol initiated polycaprolactone, 1,4-butanediol-initiated polycaprolactone, PTMEG-initiated polycaprolactone, and mixtures thereof. The hydrocarbon chain can have saturated or unsaturated bonds, or substituted or unsubstituted aromatic and cyclic groups.

Suitable polycarbonates include, but are not limited to, polyphthalate carbonate and poly(hexamethylene carbonate) glycol. The hydrocarbon chain can have saturated or unsaturated bonds, or substituted or unsubstituted aromatic and cyclic groups.

Polyamine curatives are also suitable for use in polyurethane covers. Preferred polyamine curatives include, but are not limited to, 3,5-dimethylthio-2,4-toluenediamine and isomers thereof; 3,5-diethyltoluene-2,4-diamine and isomers thereof, such as 3,5-diethyltoluene-2,6-diamine; 4,4'-bis(sec-butylamino)-diphenylmethane; 1,4-bis-(sec-butylamino)-benzene, 4,4'-methylene-bis-(2-chloroaniline); 4,4'-methylene-bis-(3-chloro-2,6-diethylaniline) ("MCDEA"); polytetramethylene oxide-di-p-aminobenzoate; N,N-dialkylamino diphenyl methane; p,p'-methylene dianiline ("MDA"); m-phenylenediamine ("MPDA"); 4,4'-methylene-bis-(2-chloroaniline) ("MOCA"); 4,4'-methylene-bis-(2,6-diethylaniline)

## 11

("MDEA"); 4,4'-methylene-bis-(2,3-dichloroaniline) ("MDCA"); 4,4'-diamino-3,3'-diethyl-5,5'-dimethyl diphenylmethane; 2,2',3,3'-tetrachloro diamino diphenylmethane; trimethylene glycol di-p-aminobenzoate; and mixtures thereof. Preferably, the curing agent of the present invention includes 3,5-dimethylthio-2,4-toluenediamine and isomers thereof, such as Ethacure® 300, commercially available from Albermarle Corporation of Baton Rouge, La. Suitable polyamine curatives include both primary and secondary amines.

At least one of a diol, triol, tetraol, or hydroxy-terminated curatives may be added to the aforementioned polyurethane composition. Suitable diol, triol, and tetraol groups include ethylene glycol; diethylene glycol; polyethylene glycol; propylene glycol; polypropylene glycol; lower molecular weight polytetramethylene ether glycol; 1,3-bis(2-hydroxyethoxy)benzene; 1,3-bis-[2-(2-hydroxyethoxy)ethoxy]benzene; 1,3-bis-{2-[2-(2-hydroxyethoxy)ethoxy]benzene; 1,4-butanediol; 1,5-pentanediol; 1,6-hexanediol; resorcinol-di-( $\beta$ -hydroxyethyl)ether; hydroquinone-di-( $\beta$ -hydroxyethyl)ether; and mixtures thereof. Preferred hydroxy-terminated curatives include 1,3-bis(2-hydroxyethoxy)benzene; 1,3-bis-[2-(2-hydroxyethoxy)ethoxy]benzene; 1,3-bis-{2-[2-(2-hydroxyethoxy)ethoxy]benzene; 1,4-butanediol, and mixtures thereof.

Both the hydroxy-terminated and amine curatives can include one or more saturated, unsaturated, aromatic, and cyclic groups. Additionally, the hydroxy-terminated and amine curatives can include one or more halogen groups. The polyurethane composition can be formed with a blend or mixture of curing agents. If desired, however, the polyurethane composition may be formed with a single curing agent.

In a particularly preferred embodiment of the present invention, saturated polyurethanes used to form cover layers, preferably the outer cover layer, and may be selected from among both castable thermoset and thermoplastic polyurethanes. In this embodiment, the saturated polyurethanes are substantially free of aromatic groups or moieties.

Saturated diisocyanates which can be used include, but are not limited to, ethylene diisocyanate; propylene-1,2-diisocyanate; tetramethylene-1,4-diisocyanate; 1,6-hexamethylene-diisocyanate ("HDI"); 2,2,4-trimethylhexamethylene diisocyanate; 2,4,4-trimethylhexamethylene diisocyanate; dodecane-1,12-diisocyanate; dicyclohexylmethane diisocyanate; cyclobutane-1,3-diisocyanate; cyclohexane-1,3-diisocyanate; cyclohexane-1,4-diisocyanate; 1-isocyanato-3,3,5-trimethyl-5-isocyanatomethylcyclohexane; isophorone diisocyanate ("IPDI"); methyl cyclohexylene diisocyanate; triisocyanate of HDI; triisocyanate of 2,2,4-trimethyl-1,6-hexane diisocyanate ("TMDI"). The most preferred saturated diisocyanates are 4,4'-dicyclohexylmethane diisocyanate ("HMDI") and isophorone diisocyanate ("IPDI").

Saturated polyols which are appropriate for use in this invention include, but are not limited to, polyether polyols such as polytetramethylene ether glycol and poly(oxypropylene)glycol. Suitable saturated polyester polyols include polyethylene adipate glycol, polyethylene propylene adipate glycol, polybutylene adipate glycol, polycarbonate polyol and ethylene oxide-capped polyoxypropylene diols. Saturated polycaprolactone polyols which are useful in the invention include diethylene glycol initiated polycaprolactone, 1,4-butanediol initiated polycaprolactone, 1,6-hexanediol initiated polycaprolactone; trimethylol pro-

## 12

pane initiated polycaprolactone, neopentyl glycol initiated polycaprolactone, PTMEG-initiated polycaprolactone. The most preferred saturated polyols are PTMEG and PTMEG-initiated polycaprolactone.

Suitable saturated curatives include 1,4-butanediol, ethylene glycol, diethylene glycol, polytetramethylene ether glycol, propylene glycol; trimethanolpropane; tetra-(2-hydroxypropyl)-ethylenediamine; isomers and mixtures of isomers of cyclohexyldimethylol, isomers and mixtures of isomers of cyclohexane bis(methylamine); triisopropanolamine, ethylene diamine, diethylene triamine, triethylene tetramine, tetraethylene pentamine, 4,4'-dicyclohexylmethane diamine, 2,2,4-trimethyl-1,6-hexanediamine; 2,4,4-trimethyl-1,6-hexanediamine; diethyleneglycol di-(aminopropyl)ether; 4,4'-bis-(sec-butylamino)-dicyclohexylmethane; 1,2-bis-(sec-butylamino)cyclohexane; 1,4-bis-(sec-butylamino)cyclohexane; isophorone diamine, hexamethylene diamine, propylene diamine, 1-methyl-2,4-cyclohexyl diamine, 1-methyl-2,6-cyclohexyl diamine, 1,3-diaminopropane, dimethylamino propylamine, diethylamino propylamine, imido-bis-propylamine, isomers and mixtures of isomers of diaminocyclohexane, monoethanolamine, diethanolamine, triethanolamine, monoisopropanolamine, and diisopropanolamine. The most preferred saturated curatives are 1,4-butanediol, 1,4-cyclohexyldimethylol and 4,4'-bis-(sec-butylamino)-dicyclohexylmethane.

Suitable catalysts include, but are not limited to bismuth catalyst, oleic acid, triethylenediamine (DABCO®-33LV), di-butyltin dilaurate (DABCO®-T12) and acetic acid. The most preferred catalyst is di-butyltin dilaurate (DABCO®-T12). DABCO® materials are manufactured by Air Products and Chemicals, Inc.

It is well known in the art that if the saturated polyurethane materials are to be blended with other thermoplastics, care must be taken in the formulation process so as to produce an end product which is thermoplastic in nature. Thermoplastic materials may be blended with other thermoplastic materials, but thermosetting materials are difficult if not impossible to blend homogeneously after the thermosetting materials are formed. Preferably, the saturated polyurethane comprises from about 1 to about 100%, more preferably from about 10 to about 75% of the cover composition and/or the intermediate layer composition. About 90 to about 10%, more preferably from about 90 to about 25% of the cover and/or the intermediate layer composition is comprised of one or more other polymers and/or other materials as described below. Such polymers include, but are not limited to polyurethane/polyurea ionomers, polyurethanes or polyureas, epoxy resins, polyethylenes, polyamides and polyesters, polycarbonates and polyacrylin. Unless otherwise stated herein, all percentages are given in percent by weight of the total composition of the golf ball layer in question.

Polyurethane prepolymers are produced by combining at least one polyol, such as a polyether, polycaprolactone, polycarbonate or a polyester, and at least one isocyanate. Thermosetting polyurethanes are obtained by curing at least one polyurethane prepolymer with a curing agent selected from a polyamine, triol or tetraol. Thermoplastic polyurethanes are obtained by curing at least one polyurethane prepolymer with a diol curing agent. The choice of the curatives is critical because some urethane elastomers that are cured with a diol and/or blends of diols do not produce urethane elastomers with the impact resistance required in a golf ball cover. Blending the polyamine curatives with diol cured urethane elastomeric formulations leads to the production of thermoset urethanes with improved impact and cut resistance.

Thermoplastic polyurethanes may be blended with suitable materials to produce a thermoplastic end product. Examples of such additional materials may include ionomers such as the SURLYN®, ESCOR® and IOTEK® copolymers described above.

Other suitable materials which may be combined with the saturated polyurethanes in forming the cover and/or intermediate layer(s) of the golf balls of the invention include ionic or non-ionic polyurethanes and polyureas, epoxy resins, polyethylenes, polyamides and polyesters. For example, the cover and/or intermediate layer may be formed from a blend of at least one saturated polyurethane and thermoplastic or thermoset ionic and non-ionic urethanes and polyurethanes, cationic urethane ionomers and urethane epoxies, ionic and non-ionic polyureas and blends thereof. Examples of suitable urethane ionomers are disclosed in U.S. Pat. No. 5,692,974 entitled "Golf Ball Covers," the disclosure of which is hereby incorporated by reference in its entirety. Other examples of suitable polyurethanes are described in U.S. Pat. No. 5,334,673. Examples of appropriate polyureas are discussed in U.S. Pat. No. 5,484,870 and examples of suitable polyurethanes cured with epoxy group containing curing agents are disclosed in U.S. Pat. No. 5,908,358, the disclosures of which are hereby incorporated herein by reference in their entirety.

A variety of conventional components can be added to the cover compositions of the present invention. These include, but are not limited to, white pigment such as TiO<sub>2</sub>, ZnO, optical brighteners, surfactants, processing aids, foaming agents, density-controlling fillers, UV stabilizers and light stabilizers. Saturated polyurethanes are resistant to discoloration. However, they are not immune to deterioration in their mechanical properties upon weathering. Addition of UV absorbers and light stabilizers to any of the above compositions and, in particular, the polyurethane compositions, help to maintain the tensile strength, elongation, and color stability. Suitable UV absorbers and light stabilizers include TINUVIN® 328, TINUVIN® 213, TINUVIN® 765, TINUVIN® 770 and TINUVIN® 622. The preferred UV absorber is TINUVIN® 328, and the preferred light stabilizer is TINUVIN® 765. TINUVIN® products are available from Ciba-Geigy. Dyes, as well as optical brighteners and fluorescent pigments may also be included in the golf ball covers produced with polymers formed according to the present invention. Such additional ingredients may be added in any amounts that will achieve their desired purpose.

Any method known to one of ordinary skill in the art may be used to polyurethanes of the present invention. One commonly employed method, known in the art as a one-shot method, involves concurrent mixing of the polyisocyanate, polyol, and curing agent. This method results in a mixture that is inhomogenous (more random) and affords the manufacturer less control over the molecular structure of the resultant composition. A preferred method of mixing is known as a prepolymer method. In this method, the polyisocyanate and the polyol are mixed separately prior to addition of the curing agent. This method affords a more homogeneous mixture resulting in a more consistent polymer composition. Other methods suitable for forming the layers of the present invention include reaction injection molding ("RIM"), liquid injection molding ("LIM"), and pre-reacting the components to form an injection moldable thermoplastic polyurethane and then injection molding, all of which are known to one of ordinary skill in the art.

It has been found by the present invention that the use of a castable, reactive material, which is applied in a fluid form,

makes it possible to obtain very thin outer cover layers on golf balls. Specifically, it has been found that castable, reactive liquids, which react to form a urethane elastomer material, provide desirable very thin outer cover layers.

5 The castable, reactive liquid employed to form the urethane elastomer material can be applied over the core using a variety of application techniques such as spraying, dipping, spin coating, or flow coating methods which are well known in the art. An example of a suitable coating 10 technique is that which is disclosed in U.S. Pat. No. 5,733, 428, the disclosure of which is hereby incorporated by reference in its entirety in the present application.

The outer cover is preferably formed around the inner cover by mixing and introducing the material in the mold 15 halves. It is important that the viscosity be measured over time, so that the subsequent steps of filling each mold half, introducing the core into one half and closing the mold can be properly timed for accomplishing centering of the core 20 cover halves fusion and achieving overall uniformity. Suitable viscosity range of the curing urethane mix for introducing cores into the mold halves is determined to be approximately between about 2,000 cP and about 30,000 cP, with the preferred range of about 8,000 cP to about 15,000 cP.

25 To start the cover formation, mixing of the prepolymer and curative is accomplished in motorized mixer including mixing head by feeding through lines metered amounts of curative and prepolymer. Top preheated mold halves are filled and placed in fixture units using centering pins moving 30 into holes in each mold. At a later time, a bottom mold half or a series of bottom mold halves have similar mixture amounts introduced into the cavity. After the reacting materials have resided in top mold halves for about 40 to about 80 seconds, a core is lowered at a controlled speed into the 35 gelling reacting mixture.

A ball cup holds the ball core through reduced pressure (or 40 partial vacuum). Upon location of the coated core in the halves of the mold after gelling for about 40 to about 80 seconds, the vacuum is released allowing core to be 45 released. The mold halves, with core and solidified cover half thereon, are removed from the centering fixture unit, inverted and mated with other mold halves which, at an appropriate time earlier, have had a selected quantity of reacting polyurethane prepolymer and curing agent introduced therein to commence gelling.

Similarly, U.S. Pat. No. 5,006,297 and U.S. Pat. No. 5,334,673 both also disclose suitable molding techniques 50 which may be utilized to apply the castable reactive liquids employed in the present invention. Further, U.S. Pat. Nos. 6,180,040 and 6,180,722 disclose methods of preparing dual core golf balls. The disclosures of these patents are hereby incorporated by reference in their entirety. However, the method of the invention is not limited to the use of these techniques.

55 The molding process and composition of golf ball portions typically results in a gradient of material properties. Methods employed in the prior art generally exploit hardness to quantify these gradients. Hardness is a qualitative measure of static modulus and does not represent the modulus of the material at the deformation rates associated with golf ball use, i.e., impact by a club. As is well known to one skilled in the art of polymer science, the time-temperature superposition principle may be used to emulate alternative deformation rates. For golf ball portions including 60 polybutadiene, a 1-Hz oscillation at temperatures between 0° C. and -50° C. are believed to be qualitatively equivalent to golf ball impact rates. Therefore, measurement of loss 65

## 15

tangent and dynamic stiffness at 0° C. to -50° C. may be used to accurately anticipate golf ball performance, preferably at temperatures between about -20° C. and -50° C.

The resultant golf balls typically have a coefficient of restitution of greater than about 0.7, preferably greater than about 0.75, and more preferably greater than about 0.78. The golf balls also typically have an Atti compression of at least about 40, preferably from about 50 to 120, and more preferably from about 60 to 100. The golf ball cured polybutadiene material typically has a hardness of at least about 15 Shore A, preferably between about 30 Shore A and 80 Shore D, more preferably between about 50 Shore A and 60 Shore D.

When golf balls are prepared according to the invention, they typically will have dimple coverage greater than about 60 percent, preferably greater than about 65 percent, and more preferably greater than about 75 percent. The flexural modulus of the cover on the golf balls, as measured by ASTM method D6272-98, Procedure B, is typically greater than about 500 psi, and is preferably from about 500 psi to 150,000 psi. As discussed herein, the outer cover layer is preferably formed from a relatively soft polyurethane material. In particular, the material of the outer cover layer should have a material hardness, as measured by ASTM-D2240, less than about 45 Shore D, preferably less than about 40 Shore D, more preferably between about 25 and about 40 Shore D, and most preferably between about 30 and about 40 Shore D. In an alternative embodiment, the cover has a hardness, as measured on the golf ball, of less than about 70 Shore D, more preferably between about 65 Shore D and about 40 Shore D, and most preferably between about 65 Shore D and about 55 Shore D. The casing, if present, preferably has a material hardness of less than about 70 Shore D, more preferably between about 30 and about 70 Shore D, and most preferably, between about 50 and about 65 Shore D.

It should be understood, especially to one of ordinary skill in the art, that there is a fundamental difference between "material hardness" and "hardness, as measured directly on a golf ball." Material hardness is defined by the procedure set forth in ASTM-D2240 and generally involves measuring the hardness of a flat "slab" or "button" formed of the material of which the hardness is to be measured. Hardness, when measured directly on a golf ball (or other spherical surface) is a completely different measurement and,

## 16

material composition of adjacent layers. It should also be understood that the two measurement techniques are not linearly related and, therefore, one hardness value cannot easily be correlated to the other.

- 5 The core of the present invention has an Atti compression of less than about 80, more preferably, between about 40 and about 80, and most preferably, between about 50 and about 70. In an alternative, low compression embodiment, the core has a compression less than about 20, more preferably less than about 10, and most preferably, 0. The overall outer diameter ("OD") of the core is less than about 1.610 inches, preferably, no greater than 1.590 inches, more preferably between about 1.540 inches and about 1.580 inches, and most preferably between about 1.50 inches to about 1.570 inches. The OD of the casing of the golf balls of the present invention is preferably between 1.580 inches and about 1.640 inches, more preferably between about 1.590 inches to about 1.630 inches, and most preferably between about 1.600 inches to about 1.630 inches.
- 10 15 The present multilayer golf ball can have an overall diameter of any size. Although the United States Golf Association ("USGA") specifications limit the minimum size of a competition golf ball to 1.680 inches. There is no specification as to the maximum diameter. Golf balls of any size, however, can be used for recreational play. The preferred diameter of the present golf balls is from about 1.680 inches to about 1.800 inches. The more preferred diameter is from about 1.680 inches to about 1.760 inches. The most preferred diameter is about 1.680 inches to about 1.740 inches.
- 20 25 30

## EXAMPLE

Three solid cores, each having an outer diameter of 1.58 inches, were formed of a composition comprising polybutadiene rubber, zinc diacrylate, zinc oxide, dicumyl peroxide, barium sulfate, and color dispersion. One core, representative of conventional technology, was used as a control. The two remaining cores were each additionally blended with 35 40 5.3 parts STRUKTOL® (Example 1) and the zinc salt of pentachlorothiophenol at 2.4 parts (Example 2). STRUKTOL® at 5.3 parts contains 2.4 parts PCTP. The specific compositions for each of the solid cores are presented below in Table I.

TABLE I

| INGREDIENT                      | CONTROL     |             |             |             | EXAMPLE 1   |             |             |             | EXAMPLE 2   |             |
|---------------------------------|-------------|-------------|-------------|-------------|-------------|-------------|-------------|-------------|-------------|-------------|
| polybutadiene rubber            | 100         | 100         | 100         | 100         | 100         | 100         | 100         | 100         | 100         | 100         |
| zinc diacrylate                 | 18          | 25          | 30          | 27          | 34          | 41          | 20          | 25          | 30          | 35          |
| dicumyl peroxide                | 0.5         | 0.5         | 0.5         | 1.8         | 1.8         | 1.8         | 0.8         | 0.8         | 0.8         | 0.8         |
| Struktol® A95                   | —           | —           | —           | 5.3         | 5.3         | 5.3         | —           | —           | —           | —           |
| zinc salt of PCTP               | —           | —           | —           | —           | —           | —           | 2.4         | 2.4         | 2.4         | 2.4         |
| zinc oxide                      | 26.5        | 24.1        | 22.2        | 5           | 5           | 5           | 5           | 5           | 5           | 5           |
| barium sulfate                  | —           | —           | —           | 16.2        | 13.4        | 10.6        | 21.7        | 19.7        | 17.7        | 15.7        |
| color dispersion                | 0.14        | 0.14        | 0.14        | 0.14        | 0.14        | 0.14        | 0.14        | 0.14        | 0.14        | 0.14        |
| <u>PROPERTY</u>                 |             |             |             |             |             |             |             |             |             |             |
| Effective Modulus (psi)         | 3800        | 6200        | 8700        | 4100        | 6200        | 7700        | 3600        | 5100        | 7400        | 9700        |
| Atti Compression COR @ 125 ft/s | 17<br>0.764 | 52<br>0.789 | 76<br>0.802 | 22<br>0.773 | 52<br>0.794 | 67<br>0.802 | 13<br>0.782 | 38<br>0.801 | 65<br>0.813 | 84<br>0.823 |

therefore, results in a different hardness value. This difference results from a number of factors including, but not limited to, ball construction (i.e., core type, number of core and/or cover layers, etc.), ball (or sphere) diameter, and the

65 It is very apparent that the addition of PCTP, in either form, increases COR, decreases compression, or both. In particular, the PCTP zinc salt (Example 2) provides comparable COR's with lower compression and/or increased

## 17

COR's with comparable (or lower) compression, both of which are desirable golf ball properties.

The halogenated organosulfur polymers of the present invention may also be used in golf equipment, in particular, inserts for golf clubs, such as putters, irons, and woods, and in golf shoes and components thereof.

As used herein, the term "about," used in connection with one or more numbers or numerical ranges, should be understood to refer to all such numbers, including all numbers in a range.

The invention described and claimed herein is not to be limited in scope by the specific embodiments herein disclosed, since these embodiments are intended as illustrations of several aspects of the invention. Any equivalent embodiments are intended to be within the scope of this invention. Indeed, various modifications of the invention in addition to those shown and described herein will become apparent to those skilled in the art from the foregoing description. Such modifications are also intended to fall within the scope of the appended claims.

What is claimed is:

## 1. A golf ball consisting of:

a core having a diameter of between about 1.54 and about 1.58 inches and a compression of between about 22 and about 50, the core comprising:

a polybutadiene rubber having a Mooney viscosity of less than about 50 and a halogenated organosulfur compound present in an amount of at least about 2.2 parts per hundred parts of polybutadiene rubber, the halogenated organosulfur compound having the formula:



where  $R_1-R_5$  are  $C_1-C_8$  alkyl groups; halogen groups; thiol groups; carboxylated groups; sulfonated groups; or hydrogen and at least one of  $R_1-R_5$  are halogen; and

a filler comprising a trans-regrind polybutadiene rubber having a trans-isomer content of between about 10% and about 60% and present in an amount of from about 5 parts to about 26.5 parts per hundred parts of cis-1,4-polybutadiene rubber; and

a cover having a thickness of between about 0.05 inches and about 0.1 inches, the cover consisting essentially of a first ionomer material and a second ionomer material;

wherein the golf ball has a coefficient of restitution of at least about 0.813 when measured at 125 ft/s.

2. The golf ball of claim 1, wherein the core has a diameter of between about 1.54 and about 1.57 inches.

3. The golf ball of claim 1, wherein the polybutadiene composition further comprises an  $\alpha,\beta$ -unsaturated carboxyl acid or a metal salt thereof, an organic peroxide, and a filler.

4. The golf ball of claim 6, wherein the  $\alpha,\beta$ -unsaturated carboxylic acid or a metal salt thereof is present in an amount greater than about 30 parts per hundred parts of polybutadiene rubber.

## 18

5. The golf ball of claim 7, wherein the  $\alpha,\beta$ -unsaturated carboxylic acid or a metal salt thereof is present in an amount greater than about 41 parts per hundred parts of polybutadiene rubber.

6. The golf ball of claim 1, wherein at least one of the first and second ionomer materials contain  $\alpha,\beta$ -unsaturated carboxylic acid groups, or the salts thereof, that have been fully-neutralized.

7. The golf ball of claim 1, wherein the halogenated organosulfur compound is present in an amount between about 2.2 parts and about 5 parts.

8. The golf ball of claim 1, wherein the first and second ionomer materials comprise copolymers or terpolymers of ethylene and methacrylic acid or acrylic acid partially- or fully-neutralized with salts of zinc, sodium, lithium, magnesium, potassium, calcium, manganese, or nickel.

9. The golf ball of claim 1, wherein the cover has a tan  $\delta$  of between about 0.07 and about 0.09 measured over the range of  $-30^\circ C$ . to  $20^\circ C$ .

10. The golf ball of claim 1, wherein the first ionomer material present in an amount between about 45% and about 55% and the second ionomer material present in an amount between about 55% and about 45%.

11. The golf ball of claim 1, wherein the core has a surface hardness and a geometric center hardness that differs from the surface hardness by between about 15 Shore D and about 20 Shore D.

12. The golf ball of claim 1, wherein the golf ball has a coefficient of restitution of between about 0.813 and about 0.823.

## 13. A golf ball consisting of:

a core having a diameter of between about 1.54 and about 1.57 inches and a compression of between about 22 and about 50, the core comprising:

a first polybutadiene rubber having a Mooney viscosity of less than about 50 and a halogenated organosulfur compound or the salt thereof, the halogenated organosulfur compound having the formula:

comprising a trans-regrind polybutadiene rubber having a trans-isomer content of between about 10% and about 60% and



where  $R_1-R_5$  are  $C_1-C_8$  alkyl groups; halogen groups; thiol groups; carboxylated groups; sulfonated groups; or hydrogen and at least one of  $R_1-R_5$  are halogen; and

a regrind filler present in an amount of from about 10.6 parts to about 19.7 parts per hundred parts of polybutadiene rubber; and

a cover having a thickness of between about 0.05 inches and about 0.1 inches, the cover consisting essentially of a first ionomer material and a second ionomer material;

wherein the golf ball has a coefficient of restitution of at least about 0.813 when measured at an incoming velocity of 125 ft/s.

**19**

14. A golf ball comprising:  
a core having diameter of between about 1.54 and about 1.61 inches and a compression of between about 22 and about 70, the core comprising:  
1,4-polybutadiene having a cis-structure of at least about 95% and a Mooney viscosity of less than about 50; and  
a filler comprising a trans-regrind polybutadiene rubber having a trans-isomer content of between about 10% and about 60% and present in an amount of from about 5 parts to about 26.5 parts per hundred parts of cis-1,4-polybutadiene rubber; and  
a cover having a thickness of between about 0.05 inches and about 0.1 inches, the cover consisting essentially of a first ionomer material and a second ionomer material;  
wherein the golf ball has a coefficient of restitution of between about 0.801 and 0.823 when measured at an incoming velocity of 125 ft/s.

**20**

15. The golf ball of claim 14, wherein the core further comprises a halogenated organosulfur compound or a metal salt thereof.
16. The golf ball of claim 15, wherein the halogenated organosulfur compound is present in an amount between about 2.2 parts and about 5 parts.
17. The golf ball of claim 15, wherein the halogenated organosulfur compound is selected from the group consisting of pentachlorothiophenol or a metal salt of pentachlorothiophenol.
18. The golf ball of claim 15, wherein the metal salt is selected from the group consisting of zinc, calcium, magnesium, sodium, and lithium.
19. The golf ball of claim 18, wherein the metal salt is zinc.

\* \* \* \* \*